

Oct. 23, 1923.

1,471,373

W. L. WOODWARD

METHOD OF MAKING SEAMLESS TUBES RICH IN ZINC

Filed April 2, 1921

Fig. 1



Fig. 2



Fig. 3



Fig. 4



Fig. 4



Fig. 5



Fig. 6



Fig. 8



Inventor  
W. L. Woodward.

By Hull Brock & West  
Atlys.

## UNITED STATES PATENT OFFICE.

WILLIAM L. WOODWARD, OF LAKewood, OHIO.

## METHOD OF MAKING SEAMLESS TUBES RICH IN ZINC.

Application filed April 2, 1921. Serial No. 458,116.

*To all whom it may concern:*

Be it known that I, WILLIAM L. Woodward, a citizen of the United States, residing at Lakewood, in the county of Cuyahoga and State of Ohio, have invented a certain new and useful Improvement in Methods of Making Seamless Tubes Rich in Zinc, of which the following is a full, clear, and exact description, reference being had to the accompanying drawings.

This invention relates to a novel method for making seamless tubes of zinc or of an alloy rich in zinc.

It is well known that cast zinc is of crystalline structure, incapable of being rolled or drawn except under special conditions within well defined limits and the object of my invention is to provide a cheap and simple method of producing a seamless tube from a cast metal tubular body, the finished product possessing ductility and malleability so that said tubes can be drawn, bent, swaged or otherwise manipulated in the course of commercial fabrication in which a bendable or drawable tube is desired.

With these objects in view the invention consists in the steps hereinafter described and set forth in the appended claims. In the drawing I have diagrammatically outlined the various steps of my process and in which Fig. 1 indicates a longitudinal section of a cast metal body of zinc or of an alloy rich in zinc; Fig. 2 is a similar view illustrating the first treatment to which said tubular body is subjected; Fig. 3 is a sectional elevation illustrating the beginning of the second treatment and Fig. 4 is a similar view illustrating the completion of the second treatment; Fig. 5 is a longitudinal sectional view of the transformed tubular body and Fig. 6 is a longitudinal sectional view of a seamless tube drawn from the transformed tubular body illustrated in Fig. 5; Figs. 7 and 8 are detailed sectional views illustrating another manner of carrying out my improved method and Fig. 9 is a still further modified form of carrying out the same.

In carrying out my invention I provide a tubular body A of zinc or of an alloy rich in zinc, said body being preferably cast in the form of a block and then bored centrally as indicated at A', but it will be understood that if desired the tubular body can be cast with the central opening, but in practice I

have found it desirable to bore the same. The cast tubular body is crystalline throughout and first of all I find it desirable to mechanically treat this cast metal tubular body to a limited extent and this I do by arranging the same upon a suitable mandrel B and subjecting it to a slight hammering operation through the medium of a hammer C operated in any suitable manner. The tubular body thus subjected to this preliminary mechanical treatment is then preferably heated to a slight degree, that is from 200 to 300 degrees F. and is then subjected to a compressive action for the purpose of breaking up the crystalline structure and causing the molecules to re-arrange themselves in such form that the transformed tubular body will be malleable and ductile and capable of being drawn out and worked in any desired manner without the application of heat, and in practice I prefer to place the tubular body A after being subjected to the preliminary and mechanical treatment and the slight heating operation within a strong incompressible shell or container D and then compress the same by means of a mandrel E having the tapered portion E' and the extended portion E<sup>2</sup>, said extended portion being of a diameter to fit loosely within the bore of the tubular body A and the mandrel from end to end, that is, the extended portion E<sup>2</sup>, the tapered portion E' and the main portion E are all very hard steel and highly polished and by applying pressure at the rear end of this mandrel and providing a suitable stop F at the opposite end of the shell and tubular body, I force the mandrel completely through the tubular body of zinc or of an alloy rich in zinc and in doing so compress the tubular body so as to reduce the thickness of the walls without materially lengthening the body as a whole, but in practice I have found that when the mandrel is forced through the tubular body, said tubular body in the reshaping, projects slightly beyond the end of the shell or container D indicated in Fig. 4. As the mandrel is forced through the slightly heated tubular body, said body will be heated somewhat more from the friction created by the passage of the mandrel and the smoothness of the surface of the mandrel facilitates the compression of the walls of the tubular body and in effecting this compression I completely transform the molecular struc-

ture of the tubular body and produce a tubular body A<sup>3</sup>, the walls of which are much thinner than the tubular body A and the bore A<sup>4</sup> thereof much larger than the bore 5 A' and the tubular body instead of being of crystalline formation is of such structure that said tubular body can be rolled or drawn out into tubular form as indicated at A<sup>5</sup> in Fig. 6 and all without the further 10 application of heat, the compressive action of the mandrel serving to break up the crystalline structure and transform the tubular body into one possessing malleability and ductility in a high degree. There are other 15 ways of accomplishing this same compressing and transforming action and in Fig. 7 I have shown a mold G in which the tubular body H is cast, there being a central core I to produce the necessary bore, a suitable 20 plate K being arranged at the bottom to prevent the metal escaping during the molding process. After the zinc or material rich in zinc has cooled to the proper extent I apply a follower L to the top or rear thereof 25 and apply strong pressure thereto, it being understood that the interior surface of the mold is highly polished and likewise the central rod and when the pressure is applied to the tubular cast metal body it is 30 forced out in the form of a tube as indicated at M and this tube thus forced out will be found to possess malleability and ductility in contradistinction to the crystalline structure of the tubular body before the compressive force is applied thereto and this cast 35 metal body is preferably subjected to the preliminary hammering or rolling operation indicated in Fig. 2.

In Fig. 9 I have shown a still further 40 modification in which the cast metal tubular body A is placed upon a suitable anvil N having a tubular rod O extending up through the central bore of the tubular body and then an inexpandible shell P having the tapering portion P' and contracted bore P<sup>2</sup> is 45 forced down over and around the cast metal body A and during this operation the walls of the cast metal body are compressed as previously described, and during this compressive operation the crystalline structure 50 is broken up and a new body is created in which the walls are not only thinner but the structure thereof possesses malleability and ductility so that the tubular body thus transformed can be readily further drawn or 55 worked in any manner similar to a tube possessing malleability and ductility.

It will be understood of course that the 60 walls of the shell P are highly polished similar to the mandrel E. It will thus be seen that I provide a simple and highly efficient

method of making seamless tubes of zinc or of an alloy rich in zinc.

Having thus described my invention, what I claim is:

1. The herein described method of making seamless tubes which consists in providing a cast tubular body rich in zinc, subjecting said cast tubular body to mechanical treatment, then heating said tubular body so treated and then subjecting the walls of said tubular body to lateral compression.

2. The herein described method of making seamless tubes which consists in providing a cast tubular body rich in zinc, mechanically treating said cast tubular body, then heating said tubular body so treated, then subjecting the walls of said tubular body to lateral compression to transform the crystalline structure of the cast tubular body 75 and provide the tubular body with walls of reduced thickness, the tubular body as a whole after such treatment possessing malleability and ductility.

3. The herein described method of making seamless tubes which consists in first providing a cast metal tubular body of crystalline structure, subjecting said tubular body to mechanical treatment, then heating said tubular body so treated, then breaking up the crystalline structure and transforming the tubular body into one possessing ductility and malleability by subjecting the walls of said tubular body to lateral compression and then drawing said tubular body 95 into a tube of reduced diameter.

4. The herein described method of breaking up the crystalline structure of a cast metal tubular body and rearranging the molecules thereof so as to provide a tubular body possessing ductility and malleability which consists in first mechanically treating said cast metal tubular body, then heating the same and finally subjecting the walls of said tubular body to lateral compression 100 and then drawing said body into a tube of less diameter.

5. The herein described method of transforming a cast metal tubular body of crystalline structure into a tube possessing malleability and ductility by breaking up the crystalline formation and rearranging the molecules which consists in first mechanically treating the cast metal crystalline tubular body, then heating the same, then subjecting the walls of said tubular body to lateral compression and finally drawing said tubular body to change the diameter thereof.

In testimony whereof, I hereunto affix my signature.

WILLIAM L. WOODWARD.